

Oct. 15, 1929.

G. M. EATON

1,731,923

HELICAL SPRING

Filed June 18, 1927



Fig. 1.



Fig. 2.



Fig. 3.



Fig. 4.



Fig. 5.

INVENTOR

George M. Eaton.

## UNITED STATES PATENT OFFICE

GEORGE M. EATON, OF PITTSBURGH, PENNSYLVANIA

## HELICAL SPRING

Application filed June 18, 1927. Serial No. 199,835.

My invention relates to helical springs, and more particularly to improved methods for their heat treatment.

In my co-pending application, Serial No. 5 192,597, filed May 19, 1927, I have shown that under service conditions more stress is inflicted on the metal at the smallest diameter of the coil than is inflicted on the metal at the largest diameter of the coil. In heat 10 treating the spring to enable it to withstand the stresses imposed by service for a reasonable length of time, it is current practice to quench the spring after hot coiling, by immersing it in a tank containing a quenching 15 medium. To hold the temperature of the quenching medium within proper limits, the medium is either circulated through a cooling system, or else cooling coils are installed in the tank. It has been found that 20 when a helical spring is immersed in a quiet body of quenching medium, the resulting physical characteristics of the steel located at the largest diameter of the coil are superior to the physical characteristics of the 25 steel located at the smallest diameter of the coil. This superiority at the outside increases as some direct function of the ratio expressed by the diameter of the rod from which the spring is made, divided by the 30 diameter of the mandrel on which the spring is coiled. It also increases as some indirect function of the space between adjacent convolutions of the coiled spring. These functions combine in limiting conditions to produce 35 a very pronounced difference between the physical characteristics of the outermost and innermost fibres of the coils. I have known of cases where by the Brinell test the hardness of the steel on the outside of the 40 coil was about twice the hardness on the inside of the coil. This is an entirely unsatisfactory condition, because in such a spring, the weakest material has inflicted upon it the highest service stresses.

Others have attempted to improve this situation by setting up a carefully directed circulation of the quenching medium, in an immersion quench, so that in the finished 45 spring the hardness of the surface of the

steel is practically uniform throughout the active coils.

The purpose of my invention is to produce a method of heat treatment whereby a still further improvement is made in the 55 ability of the spring to resist the stress concentrations to which I have referred in my above mentioned co-pending application.

In the accompanying drawings, in which like reference numbers indicate like elements, 60

Fig. 1 shows a cross section of a coil of a spring during the early stages of a quench by immersion in still oil.

Fig. 2 shows a similar cross section except that the oil is circulated. 65

Fig. 3 shows a cross section of a spring quenched in accordance with my invention.

Fig. 4 shows a vertical section through one form of quenching rig.

Fig. 5 shows a plan view, partly in section 70 on the line A—A of Fig. 4.

In my co-pending application, I have called attention to the fact that heat treatment tends to damage the metal in and adjacent to streaks. Referring to the drawings, in Fig. 75 1, the black area indicates metal which has been cooled by the action of the quench, the shading off representing a temperature gradient, and the unshaded core indicates that the metal in that location is still at practically 80 the quenching temperature.

As the metal cools, it must shrink, setting up hoop tension, unless the character of the 85 steel and of the quenching medium is such that martensite is formed in sufficient quantity so that its characteristic dilatation compensates for the temperature shrinkage. But it is current practice in the overwhelming majority of springs to aim at securing a troostitic structure, when the shrinkage mentioned will occur. The core is practically 90 incompressible, and the rod is too long and the ends are too rigid due to rapid cooling to permit of relief of pressure by axial plastic 95 flow. Therefore it is inevitable that the cooler outer shell must stretch by the amount that the existing temperature gradient forces it to shrink. It is also inevitable that this stretch must concentrate in the weakest por- 100

tions of the outer shell. These weakest portions are of two general classes.

First—The hottest portions of the shell, which are obviously at the critical inner region of the coil.

Second—Where the metal is of inferior structure, or in other words, where streaks exist.

It is at once evident that the most serious condition exists when a streak is located at the smallest diameter of the coils, where the forced opening of the streak during the hoop tension stage of the quench, will inevitably lead to premature failure, in the case of a hard worked spring.

Fig. 2 shows the cross section of a coil of a spring during the early stages of an immersion quench in which the quenching medium is circulated relative to the coils in a way that produces an equal cooling rate over the entire surface of the coil. While a superior peripheral uniformity of grain structure is secured by this type of quench, it is at once obvious that little if any improvement is effected if a streak is unfortunately located near the critical smallest diameter of the coil. Rigid hoop tension is set up over the entire perimeter of the section, and actual opening of any streak is almost inevitable, again resulting in premature failure.

Fig. 3 shows the cross section of a spring quenched in accordance with my invention. Briefly my invention consists of introducing the quenching medium axially into the space inside of the spring coils, or in passing the spring over a quenching rig where the spring surrounds the quenching medium, and then directing the quenching medium radially outward against the inner surface of the coils. Within the scope of my invention, the entire quenching may be carried out from the inside, or the early stages may be handled in this way, the completion of the quench being effected by immersion or in any other desired manner.

It will be clear to anyone skilled in the art that by cooling the critical region of the spring while regions immune from failure remain hot, I have relieved the critical region of most of the destructive hoop tension imposed upon it by quenching methods employed prior to my invention.

It is clear that quenching rigs may be devised in great variety for carrying out my invention. I have shown only one rig which is adaptable to either liquid or gaseous quenching media, in order to demonstrate that my invention is thoroughly practical. But I wish it to be clearly understood that my invention covers in the broadest sense the new process of quenching helical springs from the initiation of the quenching action to any desired stage, with a quench directed outwardly from the space inside the convolutions.

In Fig. 4 a stand pipe 1 is connected at its lower end with a supply of quenching medium 2 under any desired pressure. This supply connection is equipped with a quick acting control valve, located as may be desired, and not shown since it is obvious. The outer cylindrical surface 4 of the stand pipe 1 is machined to receive a series of pulley shaped members 5, which are all alike. The hub 6 and the rim 7 are finished off square with the bore 8, to a common axial length. The bore 8 is finished to an easy sliding fit on the stand pipe 1. The spokes 9 of the members 5 are of relatively small cross section and are arranged in angular spaced relation throughout the stack, to offer a minimum resistance to downward flow of the quenching medium. In stacking the members 5 on the stand pipe 1, a thin washer 10, of an inside diameter equal to the diameter of the bore 8 and of an outside diameter no greater than the outside diameter of the hub 11, is alternated with the members 5. This assembly provides an easily adjustable circular slit 12, in the horizontal plane, for the emission of a thin sheet of outwardly directed quench of uniform thickness. At the upper end of the stand pipe 1 is a return bend distributor 13 of approximately torus form. This distributor reverses the motion of the quenching medium which travels upward through the stand pipe 1 and downward through the members 5. The emission slits 12 are adjusted to a sufficiently narrow opening to permit the maintenance of pressure at all the emission slits, and also to secure the desired distribution among the various slits. Below the lowest member 5 is placed a closing flange 19 which is supported on a thimble 20.

The stand pipe 1 is supported by and emerges from a tank 14 in which is a body of quenching medium 15. From this tank a hot quench outlet pipe 16 connects to the suction of the pump which supplies the pressure to the quenching medium in the stand pipe. This pump and the necessary cooling facilities are not shown, as they are familiar to those skilled in the art.

Guides 17 serve to center the spring during the operation of internal quenching. A guard 18 surrounds the stand pipe, but the radial distance between the guard and the spring is sufficiently great to prevent improper internal cooling of the spring by external spatter of the quenching medium during the internal quenching operation.

In practicing my invention I enter the spring into the guides 17 from above the top of the stand pipe 1. I then open the quenching medium control valve, and drop the spring past the quenching planes and into the bath. In some cases it may be essential to cushion the fall of the spring at the bottom of its travel to prevent distortion due to its momentum. Since there are many obvious

ways of doing this, no cushioning facilities are shown.

When the desired reduction has been produced in the temperature of the spring, it is lifted out over the stand pipe. This may be done by means of hooks, or more elaborate facilities may be provided in a variety of obvious ways.

Operating under my invention, the critical inner surfaces of the coils are carried through recalescence before the spring is immersed in the bath. It is therefore evident that I have invented an improved method of quenching helical springs, which gives material protection to the critical regions during the stage of quenching in which material damage is inflicted by methods now in common use.

While I have described a specific form of my invention in some detail, and while I have referred briefly to a few other possibilities, it is obvious that a wide variety of other devices may be made and used without departing from the spirit and scope of my invention as set forth in the appended claims.

25 I claim as my invention:

1. The process of quenching helical springs which comprises introducing a quenching medium inside the coils in an axial direction and then directing it outwardly into contact with 30 the coils.

2. The process of quenching helical springs which comprises moving the successive coils of the spring past a plane of quenching medium which radiates from the axis of the 35 spring.

3. The process of quenching helical springs which comprises subjecting the same to a quenching medium acting upon the coils of the spring in a radial direction and outwardly from the axis of the spring and simultaneously subjecting the spring to movement longitudinally of its axis and in the direction of the quenching medium.

4. The process of quenching helical springs which comprises subjecting the same to a quenching medium acting upon the coils of the spring in a radial direction and outwardly from the axis of the spring, subjecting the spring to movement longitudinally of its 50 axis and in the direction of the quenching medium, and subsequently immersing the spring in a quenching bath.

In testimony whereof I have hereunto set my hand.

55 GEORGE M. EATON.